

## UNITED STATES PATENT OFFICE

2,625,477

## BLEACHING SILVER IMAGES WITH p-SULFO-PHENYL QUINONES OR p-NITROSO PHENOLS

George W. Sawdey, Rochester, N. Y., assignor to  
Eastman Kodak Company, Rochester, N. Y., a  
corporation of New JerseyNo Drawing. Application November 1, 1951,  
Serial No. 254,440

8 Claims. (Cl. 95—88)

1

This application relates to color photography and particularly to the removal of silver images in color photography.

In photographic color processes, such as those in which a colored image is formed by development with a primary aromatic amino developing agent in the presence of a coupler compound, the silver images formed in the development are generally present in the emulsion layer after the dye images are formed. These silver images are generally removed by converting them to a silver salt which is soluble or which is removed by hypo. A bath of this type containing potassium ferricyanide and potassium bromide is disclosed in Mannes, Godowsky, and Wilder U. S. Patent 2,252,718, granted August 19, 1941. A similar bath containing 50 grams of potassium ferricyanide and 20 grams of sodium chloride per liter of water to which has been added 1 to 5 grams of potassium chromate or potassium dichromate to retard the corrosive action of the bath on iron and iron alloys, has also been used.

The ferricyanide and halide bleach baths are not entirely satisfactory in that certain optical sensitizing dyes in the emulsion layer are not destroyed by them and these may cause stain in the emulsion layer. A further disadvantage is that any ferricyanide remaining in the element may be converted to iron oxide and produce a brown stain and there is also the objectionable corrosive action on stainless steel or iron alloys unless a chromate or dichromate is used in the bath.

A bleach bath containing quinone, acid and an organic solvent has also been used to convert silver images to silver salt in the presence of a developed dye image. A bath of this type is disclosed in Mannes and Godowsky U. S. Patent 2,113,329, page 2, column 2, lines 16 to 21. This bath cannot be used in the final stages of a color process because it destroys the dyes as well as converts the silver to a silver salt.

In addition to the bleaching agents described above, sodium quinone sulfonate has been suggested as a reducer for silver by Lumiere and Seyewetz (British Journal of Photography, 1910, 57 page 625). However, acid solutions of sodium quinone sulfonate lose their bleaching activity rapidly and after about six hours are for all practical purposes useless as bleaches.

It is, therefore, an object of the present invention to provide novel bleaching agents for bleaching silver images in the presence of color-developed dye images in a photographic emulsion layer. A further object is to provide a novel

method for converting silver images to a silver salt without destroying the dye images present in the emulsion layer. A still further object is to provide a bleach bath which keeps for a considerable length of time. Other objects will appear from the following description of my invention.

These objects are accomplished by bleaching the silver with a solution of p-sulfophenylquinone or p-nitrosophenol or their ring-substituted derivatives. Substituents in the aromatic rings of these compounds may include alkyl groups such as methyl, ethyl, propyl or butyl; halogen substituents such as chlorine, bromine or iodine; alkoxy substituents such as methoxy, ethoxy and propoxy; acetamido groups, etc.

P-sulfophenylquinone has the following structure:



p-Nitrosophenol is commonly regarded as existing in acid solution as the monoxime of benzoquinone according to the scheme



The bleaching agents of my invention are used in strong acid solution, that is, in a solution of pH from about 1 to about 3.5.

The bleach baths employed according to my invention may be used in any process in which silver images are present in a photographic layer together with dye images. The dye images may be those formed by color development as described in Mannes, Godowsky, and Wilder U. S. Patent 2,252,718; Mannes and Godowsky U. S. Patents 2,113,329 and 2,304,940; or Jelley and Vittum U. S. Patent 2,322,027. These dyes are of the azomethine, indoaniline or indophenol type. The dyes may also be azo dyes such as those used in the silver dye bleach process of color photography. After all of the steps of color processing, the photographic layer or element is treated with the bleach bath of my invention followed by hypo to remove the silver salts formed by the bleach bath.

The emulsion layers containing the silver and dye images treated according to my invention may be coated on supports of glass or of cellulose ester, synthetic resin, paper or other suitable material.

The following examples illustrate baths which may be used according to my invention.

*Example 1*

|                      | Grams |
|----------------------|-------|
| p-Sulfophenylquinone | 2     |
| Potassium bromide    | 5     |
| Sodium bisulfate     | 5     |
| Water to 500 cc.     |       |

The pH of this solution is approximately 1.5, which I have found to be optimal for the use of p-sulfophenylquinone, particularly when it is used with emulsions coated on paper.

*Example 2*

|                      | Grams |
|----------------------|-------|
| Cupric chloride      | 10    |
| p-Sulfophenylquinone | 2     |
| Potassium bromide    | 5     |
| Sodium bisulfate     | 5     |
| Water to 500 cc.     |       |

Both of these bleach baths effect complete conversion of silver to silver salt in a color paper or film in approximately 10 minutes.

*Example 3*

|                             | Grams |
|-----------------------------|-------|
| p-Nitrosophenol sodium salt | 4     |
| Potassium bromide           | 5     |
| Sodium bisulfate            | 15    |
| Water to 1 liter            |       |

The pH of this solution is approximately 1.0. In the majority of multi-layer color materials, complete silver bleaching is accomplished in 5 to 10 minutes.

The bleach baths of my invention have many advantages over the prior art bleaching agents mentioned above. The bleach bath may be formulated with ease since the bleaching agents are generally soluble in water. The vapors of the bleach bath are non-irritating either to the skin or nasal membranes and baths compounded according to my invention are stable and usable over long periods of time without danger of producing or increasing stain caused in the photographic layer. The baths do not react quickly or violently and therefore good control of the bleaching action may be obtained, particularly at the start of bleaching.

It will be understood that the examples included herein are illustrative only and that my invention is to be taken as limited only by the scope of the appended claims.

I claim:

1. The method of removing only the silver images from a photographic layer containing silver and dye images, which comprises treating said layer containing said silver and dye images with

an acid solution of a bleaching agent selected from the class consisting of p-sulfophenylquinone and benzoquinone monoxime and their derivatives substituted in the aromatic ring with a group selected from the class consisting of alkyl, halogen, alkoxy and acetamido groups, followed by fixing.

2. The method of removing only the silver images from a photographic layer containing silver and color-developed dye images which comprises treating said layer containing said silver and dye images with an acid solution of p-sulfophenylquinone, followed by fixing.

3. The method of removing only the silver images from a photographic layer containing silver and color-developed dye images which comprises treating said layer containing said silver and dye images with an acid solution of benzoquinone monoxime, followed by fixing.

4. The method of removing only the silver images from a photographic layer containing silver and color-developed dye images which comprises treating said layer containing said silver and dye images with an acid solution of p-sulfophenylquinone, potassium bromide and sodium bisulfate, followed by fixing.

5. The method of removing only the silver images from a photographic layer containing silver and color-developed dye images which comprises treating said layer containing said silver and dye images with an acid solution of p-nitrosophenol sodium salt, potassium bromide and sodium bisulfate, followed by fixing.

6. A bleach bath for conversion to silver salt of only the silver images in a photographic layer containing both silver and dye images, comprising an acid solution of potassium bromide, sodium bisulfate, and a bleaching agent selected from the class consisting of p-sulfophenylquinone, benzoquinone monoxime and their derivatives substituted in the aromatic ring with a group selected from the class consisting of alkyl, halogen, alkoxy and acetamido groups.

7. A bleach bath for conversion to silver salt of only the silver images in a photographic layer containing both silver and dye images, comprising an acid solution of potassium bromide, sodium bisulfate, and p-sulfophenylquinone.

8. A bleach bath for conversion to silver salt of only the silver images in a photographic layer containing both silver and dye images, comprising an acid solution of potassium bromide, sodium bisulfate, and benzoquinone monoxime sodium salt.

GEORGE W. SAWDEY.

No references cited.